

Aug. 23, 1938.

J. R. WILLARD

2,127,576

MARKING PLATE

Filed April 24, 1936



Fig. 4.



BY

INVENTOR.

JOHN R. WILLARD.

*Donald W. Robertson*  
ATTORNEY.

## UNITED STATES PATENT OFFICE

2,127,576

## MARKING PLATE

John R. Willard, New Kensington, Pa., assignor  
to Aluminum Company of America, Pittsburgh,  
Pa., a corporation of Pennsylvania

Application April 24, 1936, Serial No. 76,229

2 Claims. (Cl. 40—125)

This invention relates to improvements in marking plates and like indicia, and particularly to automobile registration plates of the so-called permanent type.

5 This type of registration plate is coming into general use and is usually characterized by having a permanent portion indicating the registration number and a replaceable portion for indicating the year for which its use is authorized by payment of an annular registration fee.

10 It is an object of the present invention to provide a registration plate of this type that is readily and economically fabricated and is also resistant to the ordinary wear and abuse to which 15 such plates are subjected. A further object is a provision of a replaceable portion that may be readily attached to the plate proper, but which can not be removed without rendering it unfit for further use. Other objects will be apparent from 20 the following specification and drawing in which:

Fig. 1 shows a registration plate constructed according to my invention having a part of the replaceable portion broken away;

Fig. 2 shows a section taken along the lines 25 II—II of Fig. 1;

Fig. 3 shows to a large scale an elevation of the replaceable portion; and

Fig. 4 shows the replaceable portion in plan.

Referring to the drawing, the reference number 30 1 indicates the main portion of the registration plate having applied thereto the registration number and the name of the State issuing the registration. In the form illustrated, two elongated apertures or perforations 2 are provided 35 below the registration number.

The replaceable portion 3 indicating the year for which the registration is authorized is provided with two lugs 4 adapted to fit in the holes 2 in the plate. Notches 5 are provided at the 40 junction of the lugs with the main body of the replaceable portion to facilitate bending.

For attachment to the plate proper the lugs are bent through an angle of approximately 90° and inserted in the openings 2 in the plate. After insertion the lugs are bent down flat as shown in Fig. 2. It is apparent that any number of such lugs can be provided on the replaceable portion of the plate and a corresponding number of apertures provided in the plate proper.

50 The main body of the plate may be made of any suitable material, but because of its permanent character is preferably made of a material which is substantially resistant to corrosive attack, such as some of the alloys of aluminum. The replaceable portion, however, should be made of a material which is easily broken upon reverse bending, so that any attempt to remove the replaceable portion after it is once fixed to the plate proper will cause the lugs to break off.

I have found that an alloy of aluminum con-

taining approximately 1.25 per cent of manganese and the balance substantially pure aluminum when subjected to a certain amount of working in the cold state to be particularly susceptible to failure when subjected to reverse bending. As the replaceable portion of a license plate is more conveniently made from rolled sheet metal, I have elected to designate the amount of cold working in the manner customarily used in sheet metal production, though its equivalent may be effected by other cold working processes.

5 I prefer to form a replaceable portion from sheet aluminum alloy of the above composition which has been subjected to a gauge reduction equal in amount to approximately the 8 Brown and Sharpe gauge numbers preceding the final gauge after the final annealing operation. If, for example, it is desired to make the replaceable portion of material having a thickness equal to No. 20 Brown and Sharpe gauge (0.032"), the 10 aluminum alloy is first rolled to a thickness equal to No. 12 Brown and Sharpe gauge (0.0808") and annealed at from 750° to 800° Fahrenheit, and subsequently rolled to the final thickness.

15 The susceptibility of the material to failure upon reverse bending is greatly augmented by providing sharply inclined notches along the line of bending. Material as above described 0.032" thick having 60° notches about 0.010" deep at the juncture of the lugs and bent as shown invariably 20 failed when an attempt was made to straighten the lugs to a position which would permit their removal from the slots.

25 What I claim is:

1. In a marking plate of the described type, a 30 replaceable portion of an aluminum alloy containing 1.25 per cent manganese, balance aluminum, and possessing the characteristics of an alloy of this composition which has been sufficiently cold worked subsequent to final annealing 35 that it is susceptible to failure upon reverse bending, said portion being provided with a plurality of lugs adapted for insertion in apertures provided in the permanent portion of the plate, and adapted to be bent into clamping relationship there- 40 with.

2. In a marking plate of the described type, a 45 replaceable portion of an aluminum alloy containing 1.25 per cent manganese, balance aluminum, and possessing the characteristics of an 50 alloy of this composition which has been subjected to cold working subsequent to final annealing in an amount equivalent to a gauge reduction of 8 Brown and Sharpe gauge numbers, said portion being provided with a plurality of lugs adapted for 55 insertion in apertures provided in the permanent portion of the plate, and adapted to be bent into clamping relationship therewith.

JOHN R. WILLARD.